

Jan. 16, 1940.

A. FORMHALS

2,187,306

ARTIFICIAL THREAD AND METHOD OF PRODUCING SAME

Filed July 28, 1937



FIG. 1.



FIG. 2.

INVENTOR.  
*Anton Formhals*  
BY  
*James A. Weber*  
ATTORNEY.

## UNITED STATES PATENT OFFICE

2,187,306

ARTIFICIAL THREAD AND METHOD OF  
PRODUCING SAMEAnton Formhals, Mainz, Germany, assignor of  
forty-five one-hundredths to Richard Schrei-  
ber-Gastell, Mainz, Germany

Application July 28, 1937, Serial No. 156,167

10 Claims.

(Cl. 18—8)

This invention relates to the production of an artificial thread, and more particularly it relates to the production of a composite thread, composed of a base thread and artificial fibers surrounding the same, by electrically spinning artificial fibers on a moving base thread.

The "electrical spinning" of artificial fibers is disclosed in U. S. Letters Patent No. 1,975,504 of Anton Formhals and comprises the electrical shattering or dispersion of a plurality of artificial fibers by means of a high electrical potential. The fibers are attracted to a moving collector electrode having a high potential charge of opposite polarity to the charge on the fibers, and during their travel to the collector electrode the solvent is evaporated from the fibers so formed.

It is the object and purpose of this invention to prepare a composite yarn or thread composed of a base thread surrounded by a plurality of electrically spun, artificial fibers.

It is another object of this invention to electrically shatter or disperse a stream of spinning solution to a plurality of fibers and simultaneously collect the same on a base thread.

Other objects of the invention will appear hereinafter.

The objects and purposes of the invention will be more clearly apparent by reference to the following description taken in connection with the accompanying drawing, in which:

Figure 1 is a diagrammatic, side elevational view of one form of apparatus for carrying out the present invention;

Figure 2 is a diagrammatic, side elevational view of a modified form of apparatus for carrying out the present invention.

Referring to Figure 1 of the drawing, reference numeral 11 designates a storage receptacle containing a quantity of spinning solution. A header conduit 13 is connected to the storage receptacle 11, and is provided with a plurality of nozzles 15 through which a stream of spinning solution is extruded. A base thread 19 which may be composed of cotton, wool, linen, hemp, artificial silk, wire, or any other desired material is passed about two grooved pulleys 23 and 25. Pulley 25 may be rotated by means of a motor 27 or in any other desired mechanical or manual method. A conductor wire 21 is positioned below the base thread 19, and the nozzles 15 are preferably positioned above the said base thread. It is preferred that the nozzles be positioned somewhat to one side of the thread 19 or conductor wire 21 and not directly over the same to prevent drip-

ping of spinning solution on the thread or wire when the electric current is shut off. One pole of an electric device 17 for the production of high potential electricity is connected to the header line 13, and the opposite pole of the device 17 is connected to the conductor wire 21. In this way there will be a high electrical potential between the nozzles 15 and the conductor wire 21. As the spinning solution is extruded in streams from the nozzles 15, they are electrically shattered by means of the high electrical potential into fine, artificial fibers which are attracted towards the oppositely charged conductor 21. As the artificial fibers are moving towards the wire 21 they will come in contact with the base thread 19 which is being moved between the nozzles and the conductor wire. The fine fibers are found to adhere to the base thread and will be collected and carried away therewith. It is found that the artificial fibers adhere quite well to the base thread and will be rolled on to the same to have close contact therewith by means of the grooved pulleys 25 and 23. The base thread as shown in Figure 1 is endless and may be moved at a desirable speed about the pulleys 23 and 25 until it has been covered with the desired depth of artificial fibers.

After the base thread has been covered with artificial fibers to the desired extent, it can be cut and tied to similar threads which have been covered with artificial fibers and the whole passed through a twisting machine whereby to give a desired twist to the composite thread. It may also be desired in certain cases to twist together a number of the composite threads to make a 2, 3 or greater ply strand or cord as may be desired.

Referring to Figure 2 of the drawing, the base thread 33 is pulled from a spool 35 positioned on a stationary support 37. The spool is preferably provided with a smooth, round edged guide member 39, and from there the base thread 33 passes through a guide 41 into contact with a moistening mechanism 43. The moistening mechanism 43 is adapted to apply to the thread a sizing composition of any desired nature, or it may be used to moisten the thread with acetone or other electrically conducting liquid so that the base thread 33 will become electrically conductive and serve as a collecting electrode. One pole of a source of high potential electricity 17 is connected to a member 34, such as a trolley or the like, which will continually contact the moving base thread 33. The trolley is preferably positioned on an insulated support 34 so as to prevent leakage of the electrical current 55.

therefrom. The opposite pole of the source of high potential electricity 17 is connected to the header 13, leading from the storage receptacle 11. The conduit 13 is provided with a large plurality 5 of nozzles 15 through which streams of spinning solution are extruded. As in the case of the modification discussed above with reference to Figure 1, the spinning solution is shattered by dispersing the same into a plurality of fine fibers 10 which are attracted to the electrically charged base thread 33. The base thread 33 is passed about the guide roll 45 and is preferably passed over a plurality of grooved rollers 47 so that the artificial fibers which are being collected on the 15 base thread in large quantities will be suitably rolled in contact with the thread so as to produce a desirable composite product. Inasmuch as the thread in this case is provided with a suitable conducting fluid, it will be unnecessary to provide 20 the apparatus with a conductor wire as in the case of Figure 1. However, this feature of the invention is purely optional and instead of moistening the thread and passing the high potential current directly on to the thread, a conductor wire such as 21, illustrated in Figure 1, may be substituted therefor. If desired, the base 25 thread containing the artificial fibers in contact therewith may be passed over a guide roller 49, through a stationary guide 51, and directly 30 through the rings 53 of a ring twisting device 55 such as is well known in the art. The thread will be twisted and directly wound upon a spool 57.

The high potential electric current used in carrying out the present invention may be constant 35 direct, fluctuating direct, or alternating current. In the case of direct current, the fibers formed will be substantially straight and will pass without any interruption directly towards the base 40 thread on which they are collected. In the case of alternating current the stream of spinning solution, during its shattering into artificial fibers, will be given slight impulses corresponding to the period of the cycle of the alternating current and thereby cause a crimp to be imparted to the fibers 45 formed, and therefore after collection by the base thread, will form a slightly different appearing composite thread from that produced by the use of direct current.

The artificial fibers may be produced from any kind or type of liquid spinning solution which will conduct an electric current and which will coagulate or harden in a fiber form. Thus, for example, artificial fibers may be formed from cellulose derivative compositions, from various resins, vitreous materials, or the like.

Particularly desirable results have been obtained by use of a spinning solution consisting of 150 parts by weight of cellulose acetate, 600 parts by weight of acetone and 300 parts by weight of monomethyl ether of ethylene glycol, and which spinning solution has a viscosity at 25° C. of about 35.7 poises. The spinning solution is preferably extruded from nozzles having 65 single orifice openings of approximately 0.0180 inch in diameter.

It may also be desirable to provide the electrical spinning apparatus with suitable field directing or shaping screens, wires or the like as described 70 in my copending application Serial No. 88,430, filed July 1, 1936, now Patent No. 2,160,962. The field directing means may be parabolically shaped or otherwise shaped to direct the fibers along a narrow path against the base thread. The spinning apparatus may also, if desired, be pro-

vided with a spark gap means to regulate the length of the fibers as disclosed in my copending application Serial No. 96,225 filed August 15, 1936, now Patent No. 2,109,333.

The base thread may have the same or a different color from the artificial fibers so as to give any desirable contrast to the finished product. The spinning solution furthermore may contain deflustering agents, pigments, dyes, or any other material to impart any desirable optical appearance to the finished product.

The present invention has particular utility in making thread composed of mixed fibers, such as for example wool fibers and cellulose acetate fibers so as to produce a product having the desirable characteristics of both kinds of threads. If desired, the wool base thread may be in the form of a sliver and after the collection of the artificial fiber, the resulting composite sliver may be drawn and twisted so as to produce a mixed 20 thread of great uniformity and very desirable characteristics.

It has also been found that a wire base thread may be covered with artificial fibers as a means of insulating the same. In this case it is often found desirable to spray the fiber coated wire with a solution of a solvent such as acetone or the like so as to cause a good, firm adherence of the artificial fibers thereto.

Since it is obvious that many changes and 30 modifications can be made in the above described invention without departing from the nature and spirit thereof, it is to be understood that the invention is not to be limited except as set forth in the appended claims.

I claim:

1. In a process for the production of a thread composed of mixed fibers, the step which comprises electrically shattering or dispersing a stream of spinning solution into a plurality of fibers on to a preformed moving base thread thus to form a composite thread.

2. In a process for the production of a thread composed of mixed fibers, the steps comprising electrically shattering or dispersing a stream of spinning solution into a plurality of fibers between two electrodes, and passing a preformed base thread between said electrodes in such a manner as to collect said fibers thereon and thus to form a composite thread.

3. In a process for the production of a thread composed of mixed fibers, the steps comprising creating a high electrical potential between a spinning nozzle and a preformed moving base thread, and passing a spinning solution through said nozzle whereby to electrically shatter and precipitate the same and cause the same to be collected on said base thread and thus to form a composite thread.

4. In a process for the production of a thread composed of mixed fibers, the steps comprising electrically shattering or dispersing a stream of spinning solution into a plurality of fibers on a preformed moving base thread, and mechanically pressing said fibers on the said base thread to form a composite thread.

5. In an apparatus for the production of a thread composed of mixed fibers, a spinning nozzle, an electrical conductor spaced from said nozzle, means for connecting opposite poles of a source of high potential electricity to said nozzle and conductor and means for moving a base thread adjacent said conductor.

6. A composite thread comprising a base thread

and a surrounding covering of artificial fibers electrically spun onto said base thread.

7. A composite thread comprising a base thread and a surrounding covering of artificial fibers electrically spun onto said base thread said fibers positioned substantially longitudinally of said thread.

8. A composite thread comprising a base thread and a surrounding covering of fibers electrically spun onto said base thread, said fibers twisted into close contact with said base thread.

9. In a process for coating a preformed long narrow object of substantially uniform cross-section such as a wire, thread or the like, the steps which comprise electrically shattering or dispersing a stream of spinning solution into a

plurality of fibers and simultaneously collecting the same on said object while moving the latter along a predetermined path and then collecting the thus formed composite, thread-like member.

10. In a process for coating a preformed long narrow object of substantially uniform cross-section such as a wire, thread or the like, the steps comprising electrically shattering or dispersing a stream of spinning solution into a plurality of fibers between two electrodes, passing said object between said electrodes along a predetermined path in such a manner as to collect said fibers thereon and then collecting the thus formed composite, thread-like member.

ANTON FORMHALS. 15